

April 21, 1925.

W. HOOPES ET AL

**1,534,319**

## REFINING ALUMINUM ELECTROLYTICALLY WITH FUSED ELECTROLYTES

Filed Dec. 21, 1922



Patented Apr. 21, 1925.

1,534,319

# UNITED STATES PATENT OFFICE.

WILLIAM HOOPES, OF PITTSBURGH, AND FRANCIS C. FRARY, OF OAKMONT, PENNSYLVANIA, ASSIGNEES TO ALUMINUM COMPANY OF AMERICA, OF PITTSBURGH, PENNSYLVANIA, A CORPORATION OF PENNSYLVANIA.

## REFINING ALUMINUM ELECTROLYTICALLY WITH FUSED ELECTROLYTES.

Application filed December 21, 1922. Serial No. 608,286.

To all whom it may concern:

Be it known that we, WILLIAM HOOPES and FRANCIS C. FRARY, both citizens of the United States of America, the said WILLIAM HOOPES residing at Pittsburgh, and the said FRANCIS C. FRARY residing at Oakmont, both in the county of Allegheny and State of Pennsylvania, have invented certain new and useful Improvements in Refining Aluminum Electrolytically with Fused Electrolytes, of which the following is a full, clear, and exact description.

This invention relates generally to electrolytic refining, particularly of aluminum, by removal or separation of the metal from an alloy or a mixture thereof with other substances, and relates more particularly to a refining process in which the electrolyte floats, in a molten state, upon the molten alloy; the latter being used as anode and the aluminum removed being deposited on a layer of molten aluminum as cathode floating on the electrolyte.

In an extensively used aluminum reduction process, wherein aluminum is produced by reduction of its oxid, a cryolite bath or electrolyte is used, but in the herein described process, in which it is desired to have the refined metal float on the electrolyte, such a bath, though otherwise operable, can not be used alone for the purpose, since in the molten state it is lighter than aluminum and hence would allow the latter to sink. While other salts may be added to give adequate density, such addition easily leads to difficulties of various sorts, resulting in failure to produce pure metal, and no prior inventor, so far as we are aware, has attained commercial success in this way or in any other. We have found that success may be realized and a bath produced combining the desired characteristics of density, fluidity, stability, capacity for dissolving alumina, conductivity, and selective solution and deposition of aluminum during electrolysis, by adding to cryolite (or preferably to a mixture of aluminum and sodium fluorides richer in aluminum fluorid than is cryolite) salts of the alkali earth metals. These metals are less easily precipitated from the bath than aluminum and we find certain of their salts to be the only generally available materials suitable for the purpose of increasing the density of the bath. We

find that the only materials giving in high degree the other necessary or desirable characteristics are the fluorids of these metals (barium, strontium, calcium and magnesium). These form with cryolite, mixtures which are readily fusible, but experience indicates that magnesium fluorid has less effect than any of the others in increasing the density of the bath. Barium fluorid has been suggested as an ingredient of electrolytes for other purposes, but so far as we are aware no one has heretofore suggested their use for aluminum refining, or has given, with respect to the properties of barium fluorid and cryolite mixtures, the information needed for their successful use. It has been found, however, that within certain limits, mixtures of the substances mentioned furnish excellent electrolytes, and that such a bath does not lose aluminum fluorid by volatilization at the working temperature to a serious extent. Its electrical conductivity and power of dissolving alumina are also good.

As stated in the copending application of William Hoopes, Francis C. Frary and Junius D. Edwards, Serial No. 608,285, filed Dec. 21, 1922, the density of aluminum of 99.75 per cent purity is approximately 2.29 grams per cc. at 1000° C. At this temperature, the density of molten cryolite is approximately 2.10 grams per cc. In order to increase the density of the cryolite, so that this aluminum will float on it at the temperature mentioned, we have found that there must be added about 20 parts of barium fluorid to each 80 parts of cryolite. If calcium fluorid were to be used, about 40 parts would be required to 60 parts of cryolite. While the above mentioned mixture of cryolite and barium fluorid is completely fluid at temperatures above 965° C., mixtures of calcium fluorid and cryolite containing about 40 per cent or more of the former by weight require a temperature above 1000° C. to keep them fluid. This would make the working temperature of the bath undesirably and in some cases impracticably high. On the other hand, mixtures of cryolite and one or more fluorids of alkali earth metals having atomic weights above 80 are in general suitable; though of course radium is to be excepted, for obvious reasons. Thus mixtures of cryolite and barium

fluorid containing between about 20 and 60 per cent of the latter constituent by weight are readily fusible at temperatures below 1000° C., and have densities in the molten state ranging between about 2.38 and 3.15 grams per cc. at 1000° C. Even the heaviest of these mixtures is sufficiently light to float on any of a number of molten aluminum alloys suitable for use as anode in the electrolytic refining of aluminum.

A fused mixture of cryolite and strontium fluorid containing between about 20 per cent and 60 per cent of the latter lies within the proper range of densities for our purpose, but such mixtures containing more than about 40 per cent of strontium fluorid are in general not so readily fusible as mixtures containing corresponding amounts of barium fluorid.

In operating with a bath of the type described above, it has been observed that there is a considerable deposition of metallic sodium at the cathode, and that this sodium, being in vapor form, passes up through the molten aluminum cathode, and accumulates in the crust which forms above, where it causes difficulties in connection with the leading out of the current from the cathode metal. Carbonaceous rods used to carry the current out of the floating layer of aluminum are attacked and eventually disintegrated by the sodium, but we have found that this difficulty may be decreased, without interfering seriously with the density of the molten bath, by increasing the proportion of aluminum fluorid as compared to sodium fluorid, although such an increase does perceptibly increase the electrical resistance of the bath.

As an example of baths or electrolytes which have been found by actual use to be suitable we recommend the one described and claimed in the above mentioned application of ourselves and Junius D. Edwards, Serial No. 608,285. This bath has approximately the following composition:

|                                                                            | Per cent. |
|----------------------------------------------------------------------------|-----------|
| Barium fluorid                                                             | 30 to 38  |
| Sodium fluorid                                                             | 25 to 30  |
| Aluminum fluorid                                                           | 30 to 38  |
| Alumina                                                                    | 0.5 to 3  |
| Calcium and magnesium fluorid<br>(present as unavoidable impurities) about | 2         |

Such a bath is completely molten at all temperatures above 900° C. and enables the refining to be carried on at about 950° C. At this temperature the bath is satisfactorily stable, has good electrical conductivity and satisfactory density, and may dissolve as much as 7 per cent of its weight of alumina.

It will be understood that the sodium and aluminum fluorids of the electrolyte may be supplied, in part at least, by cryolite, which has a composition generally accepted as  $3\text{NaF} \cdot \text{AlF}_3$ .

It has been observed that the density of these molten baths decreases more rapidly with rising temperature than does the density of the molten aluminum, and hence it is advantageous to provide a distinct margin of safety between the two densities, so that if the cell should become overheated the bath will not become so light as to permit the aluminum top layer to sink to the bottom. The density of a bath of the above mentioned composition lies between about 2.5 and 2.7 at 950° C., and between about 2.4 and 2.6 at 1100° C., and accordingly pure aluminum will float on the bath at these temperatures, since the density of aluminum at 950° C. is about 2.30, and at 1100° C. is about 2.26 grams per cc.

An electrolyte composed of cryolite saturated with alumina, and another composed of cryolite and barium chlorid have been suggested heretofore, but we have found that the addition of alumina to cryolite actually decreases rather than increases the density. The addition of barium chlorid does increase the density of the bath but not so rapidly as does the addition of fluorid of calcium, strontium or barium. However, a bath composed of 40 per cent barium chlorid and 60 per cent cryolite has a density such that at 1000° C., aluminum of a purity of 99.75 per cent will barely float on it, but if the temperature be raised to 1050° C. its density decreases to such an extent that it is then lighter than aluminum and the latter will therefore sink. In order to obtain a density of about 2.48 at 1000° C., which would give a density-difference of about 0.19 between the bath and the aluminum at 1000° C., and a difference of about 0.17 at 1050° C., it would be necessary to use a mixture of about 60 parts barium chlorid and 40 parts cryolite.

While the freezing points of such mixtures are advantageously low, they labor under the disadvantages of producing an excessive amount of fumes at temperatures in the neighborhood of 1000° C., and of being poor solvents of alumina. Thus the above mentioned bath containing 60 per cent barium chlorid can dissolve only about 1 per cent of alumina. On the other hand a bath containing cryolite and 60 per cent barium fluorid (instead of the chlorid) will dissolve between 4 and 5 per cent of alumina; and a similar bath containing 40 per cent barium fluorid, which would have a specific gravity of about 2.73 will dissolve between 8 and 9 per cent of alumina at 1000° C. Electrolytes of such type are therefore advantageous for the following reasons.

Alumina becomes more soluble in any of the cryolite baths as their temperature is raised, but if alumina be added until the bath is saturated it will be found that a

small drop in temperature will cause some of the alumina to precipitate out as corundum or in corundum-like form, with which more or less bath will be mechanically associated. In an operating cell the portion of the bath adjacent to the walls, together with that portion forming the top crust or coming in contact with it, is at a temperature distinctly lower than that of the main body of the bath, so that if sufficient alumina enters to saturate this main body the natural circulation will cause a deposition of part of the alumina on the walls of the cell in the form of a thickened crust. Practical operation of such a bath has shown that when the alumina has once crystallized in this form, it is extremely difficult to re-dissolve it in the bath. A certain amount of such crust on the interior of the cell is desirable for its thermal and electrical insulating properties (as described more fully in the copending application of William Hoopes, Junius D. Edwards and Basil T. Horsfield); but to prevent the formation of an undesired amount of this deposit, which would otherwise gradually fill up the cell and interfere with the operation, it is important to keep the alumina content below the saturation point. In order to maintain this condition it is therefore desirable, in practice, to have the bath capable of dissolving considerable alumina, so as to allow for unavoidable variations incident to operating conditions; for the reason that any of the following causes may operate to add alumina to the baths: (A) The hydrolysis of aluminum fluorid by moisture. Capillary action continually brings some of the bath up between the top metal layer and the side of the cell, so that it forms a crust on the top of the metal, where it is maintained at a high temperature and exposed to the air. The excess of bath above that which can solidify to form this crust drips back through the metal from time to time, and when the crust is disturbed or broken, parts of it sink through the metal, and return to the main body of the bath. (B) The reaction of sodium oxid (or hydroxid) with aluminum fluorid. More or less sodium is always liberated at the cathode, and some of it rises through the metal layer, probably in the form of vapor, and reaches the top crust where it is oxidized by contact with the air. (C) The direct oxidation of the floating aluminum layer by air penetrating through cracks in the top crust. (D) Alumina dust, which is always present in a plant in which the Hall process of producing aluminum is operated, will settle on the crust of the refining cell if it is operated in the same plant.

So important is it to have the bath unsaturated that in actual commercial operation it is generally necessary to remove

alumina from time to time. This may be conveniently done in various ways, as by one or another of the methods described herein-after.

The cell preferred for use in the present process of refining aluminum is of the type described and claimed in copending application of William Hoopes, Serial No. 608,287 filed December 21, 1922. One form of this cell, with the addition of means for reducing the alumina content of the bath, is illustrated in the drawings annexed hereto, in which—

Fig. 1 is a plan view of the cell.

Figs. 2 and 3 are cross sections on lines 2—2 and 3—3, respectively, of Fig. 1.

Figs. 4 and 5 are detail cross sections on lines 4—4 and 5—5, respectively, of Fig. 1, illustrating the water connections to and from and between the water jackets.

Fig. 6 is a detail cross section on line 6—6 of Fig. 1, showing the method of connecting the upper electrodes to the negative busbars.

Fig. 7 is a detail cross section on the same plane as Fig. 2, illustrating the method of securing the upper and lower shell sections together to give adequate mechanical strength without connecting the two electrically.

Fig. 8 is a detail sectional view illustrating a suitable anode for use in deoxidizing the electrolyte.

Fig. 9 is a detail sectional view on the same plane as Fig. 2, illustrating the refractory electrically and thermally insulating crust which is produced and maintained above the molten cathode layer.

The lower shell or shell section 10 is preferably made of steel in the form of a cylindrical vessel of considerably greater diameter than height, and at or near its top it is provided with a water jacket 11 which is most conveniently formed by providing at the upper edge of the shell section an outwardly extending flange 12 of suitable width, and a flaring or conical ring 12a welded or otherwise hermetically joined to the underside of the flange and to the body of the shell below.

Above the lower shell section 10 is an upper shell section 13 which may also be of steel and formed with hollow walls to provide an upper water jacket 14. The inner surface of the upper shell section is preferably flaring, as indicated. To keep the sections electrically insulated or separated from each other a flat ring or gasket 15, of asbestos or other suitable material, may be used between the two.

In order to give the shell structure sufficient mechanical strength the sections may be secured together by means of machine studs 16 passing upwardly through the flange 12 and threaded into pads 17 welded on the bottom of the upper shell inside the

water jacket. To prevent electrical connection the holes in the flange 12, through which the studs pass, may have insulating bushings 18 and insulating washers 19 may be used. If the water jackets are used, as in most cases they will be, the bushings and washers will not be subjected to a high temperature and hence they can be made of practically any insulating material which will not soften at temperatures below 100° C. and which can withstand the crushing stress exerted by the studs. Mica has been found satisfactory for the purpose.

Suitable water connections for the water jackets are provided, and for the sake of simplicity and convenience these connections may be so constructed and arranged that the water flows through the two jackets in succession, preferably through the lower jacket first. For this purpose the jacket 11 may be provided at the bottom with an inlet nipple 20 connected by a pipe 21 to any convenient source of water, not shown, and at the top (to prevent pocketing of air) with an outlet nipple 22 connected by a pipe 23 to the inlet nipple 24 by which water from the lower jacket is led into the bottom of the upper. The latter is equipped with an outlet nipple 25 (at the top to prevent air pocketing) which may be connected to a waste pipe 26 by means of a pipe 27. To avoid electrical grounding the pipes 21 and 27 may consist of rubber hose, as may also the pipe 23 to keep the two shell sections electrically separate. The water used when the jackets are connected should be of sufficient purity to prevent material flow of current from one shell section to the other at the voltage employed in operation.

In the bottom of the lower shell section a layer 28 of heat-insulating material may be provided, as powdered bauxite, alumina, magnesia, or refractory bricks, to decrease or minimize loss of heat through the bottom of the cell, and above this layer is a bottom lining 29 of refractory electrically conducting material, preferably carbon, and preferably having a cavity or depression in its upper portion to receive the alloy or other material to be refined. The bottom lining can be conveniently and satisfactorily made by tamping into the shell a mixture of tar, pitch and granular or powdered coke, at a temperature high enough to make the mass plastic, and placing the shell and contents in an oven in which the temperature is gradually raised, say to about 600° C., for the purpose of baking and solidifying the carbonaceous mass.

Good electrical connection may be provided between the shell and its bottom lining by means of metal collector plates 31, welded to the inner surface of the shell so as to be electrically and mechanically continuous therewith. These plates extend in-

wardly into the bottom lining, which is molded around them. At the plane of the collector plates the shell may be provided on the outside with metal contact pads 32, preferably welded to the shell so as to be mechanically and electrically continuous therewith, to which pads busses or busbars, of copper, aluminum or other suitable metal may be bolted tightly in place. The busbars may be in the form of long flat plates 33 embracing the lower shell section, with their ends brought out at one side of the cell for convenient connection to one terminal of a suitable source (not shown) of continuous or unidirectional current. During the refining operation these busses are connected to the positive terminal or pole of the source, so that the current enters the cell at the bottom. The carbon bottom or bottom-lining, 29, constitutes what may for convenience be termed the lower electrode of the cell.

The upper electrode may be multiple, as indicated, composed preferably of a suitable number of short thick rods 34 of graphite, arranged vertically and having 90 copper or other metal rods 35 threaded or otherwise suitably secured to the tops of the electrodes. These metal rods serve to support the upper electrodes and convey current to or from the same, and for this purpose they may be releasably and adjustably secured, as by means of clamps 36, to metal busbars 37 extending horizontally across the cell. For convenience of access to the electrodes, for adjustment, replacement, etc., the busbars may be arranged at two or more different levels, as indicated, and may be supported on and secured to a plurality of legs 38 to form a rigid framework. The latter may rest on the upper shell section, in which case they are insulated from the shell section, as by any convenient and suitable means, not shown.

It is recognized that, strictly speaking, the aluminum layer floating on the bath 110 and the layer of alloy underlying the bath, are the upper and lower electrodes, respectively, but these layers are termed herein the cathode and the anode, and hence it is deemed permissible as well as convenient to 115 refer to the graphite cylinders and the carbon bottom-lining, or their equivalents, as the upper and lower electrodes.

Metal or other molten material may be withdrawn from the upper portion of the cell through a tapping notch 39, which may be closed by means of any suitable refractory material. Molten metal or other material may be withdrawn from the lower part of the cell through a port or tapping hole 40, which may be closed by means of a plug of dense charcoal.

On the inside of the cell is a side-lining 45 extending upwardly from the carbon bottom 29, over the joint between the shell 130

- sections and well up toward or even over the top of the upper shell section. This side lining should be thermally and electrically insulating, to decrease or minimize the conduction of heat to the water jackets as well as to prevent by-passing of current around any part of the cell contents undergoing electrolytic treatment in the refining operation. The lining should also be refractory enough to remain solid at the temperatures to which it is subjected in the electrolytic refining operation. Under these conditions a lining composed of or formed from a mixture of metal fluorides and aluminas, as more fully explained in the above mentioned application of Hoopes, Edwards and Horsfield, has been found highly satisfactory in practice.
- In the refining process the aluminum alloy or mixture of aluminum and other substances lies in molten form in the bottom of the cell as indicated at 46. Floating on this is a layer 47 of fused bath or electrolyte, and on the latter is a layer 48 of molten aluminum, with the upper electrodes extending into it far enough to insure good electrical contact. The molten layers are preferably established in the cell by successively pouring the previously fused materials into place, using for the original aluminum layer the purest metal conveniently available. The cell, however, may be also put in operation in the following manner.
- The upper electrodes are lowered into contact with the carbon bottom and current is sent through them to the latter, thereby generating heat and fusing a small quantity of powdered or granulated bath material placed around them. The upper electrodes are raised as the melting proceeds, and additional bath material is supplied, until a sufficient body of fused electrolyte has been produced. The molten anode alloy or mixture is then poured in. Almost any aluminum alloy can be used which is denser than the molten bath and which will remain mobile during the refining operation. It should be supplied in sufficient amount so that it will remain in an electrically continuous layer on the bottom of the cell throughout the refining operation. A bath layer of sufficient depth should be used so that the top metal (the pure aluminum) will in no case come into contact with any portion of the side crust which has previously been covered by the anode alloy. It is to be noted in this connection that the changes in composition of the anode alloy, incident to the refining operation, cause corresponding changes in its volume and in the position of the upper and lower surfaces of the bath layer. Molten aluminum, preferably the purest obtainable, is placed on the molten bath, to serve as cathode.

The refining process can now be begun, with the alloy as anode and the top metal as cathode, the current being led from the top metal by means of graphite electrodes dipping into it. Under these conditions aluminum is dissolved out of the anode alloy and deposited in molten form on the cathode. This is continued until the desired amount of aluminum has been removed from the anode and added to the cathode. A portion of the top metal is then removed and the impoverished anode alloy is withdrawn through the tap hole 40, fresh anode alloy in the molten state being supplied in any convenient way, preferably such that the refined metal floating on the bath will not be contaminated. This operation may be conveniently performed by means of a carbon funnel, which, after being preheated, is let down until it nearly reaches the bottom of the cell, which has preferably been cut out of the circuit. The refined metal entrapped in the funnel may be dipped out with a hand ladle, after which the fresh anode alloy is poured in. The funnel is then lifted out and the refining process resumed. The fresh anode alloy introduced is preferably sufficient in amount to raise the bath and top metal until the surface of the latter is at the same level as before the withdrawal. These operations may be repeated from time to time as necessary or desirable without seriously interrupting the refining process, which otherwise can go on continuously.

Notwithstanding the greater density of the bath, a portion of it is carried up by capillary action at the area of contact between the liquid aluminum and the solid boundary crust and rises to the surface of the former, where it spreads in a thin layer, the weight of which is insufficient to overcome the surface tension of the liquid aluminum. Consequently it spreads over the entire surface of the latter, and by reason of the escape of heat into the air, solidifies there, forming a top-crust such as indicated, for example, at 58 in Fig. 9. This process goes on until the crust thickens so much that (the escape of heat being thus retarded) the temperature of its under surface can rise to the melting point of the bath. When this thickness is attained, quantities of unsaturated bath subsequently carried up by capillary action can accumulate in liquid form under the crust and finally grow to a mass of sufficient dimensions to be able to sink through the aluminum. Hence, if the bath is kept unsaturated with alumina, the top crust forms up to a certain thickness, after which its growth ceases. On the other hand if the freezing point of the bath is raised by allowing it to become saturated, liquid bath finding its way to the under surface of the crust partially solidifies there and increases the thickness. This action would,

if unchecked, result eventually in bringing up a large portion of the bath from below the aluminum and causing it to attach itself to the top crust. At the same time the boundary crust at the sides of the cell thickens as previously described, and the net result would ultimately be more or less complete solidification of the bath. Moreover, if the alumina content of the bath is too high a crust of greater or less extent is apt to form between the bath and the cathode, or between the bath and the anode, or in both these places. In most cases the crust is attached to the cell lining, and extends inwardly somewhat in the manner of a shelf. In general, such a crust is objectionable, as will be pointed out more fully hereinafter. For the above reasons it is desirable to keep the bath unsaturated in the normal operation of refining.

The bath crust formed on the aluminum layer as above described serves as a convenient and good heat insulating medium to minimize loss of heat from the top of the cell, so that a cell cover or lid of metal, refractory brick, or the like, is in general unnecessary and hence can be omitted, thus eliminating the difficulties and disadvantages incident to the use of a cover. The crust described entraps sodium as already explained, with consequent increase of alumina in the bath, but the amount of sodium which thus escapes from the bath can be minimized by using in the latter the highest permissible amount of aluminum fluorid.

Instead of forming the heat-insulating top crust in the manner hereinbefore specifically described, such a crust may be produced by dusting over the upper surface of the aluminum layer, soon after it is put in place, a layer of finely divided alumina, carbon, magnesia, or other suitable powdered material. This layer of finely divided material is rapidly cemented together by the liquid bath coming up from below and wetting it. The heat insulating property of the top crust may be increased by dusting any suitable powdered material over it after it has been formed, so that it is covered by a layer of such material, which is an excellent insulator by reason of its porous condition. Being supplied to the surface of the top crust after the latter has solidified, the additional heat-insulating material is not cemented together and therefore retains its porosity. In general, the best material for the purpose is powdered bath, since if any of it accidentally or incidentally finds its way below the top metal it does not contaminate the electrolyte.

Mention has been made herein of a crust that may form between the bath and the cathode metal, and between the bath and the anode alloy. In the latter case the area of contact between bath and anode is dimin-

ished, with the result that the current density at the active anode surface is increased. Too high a current density at the anode surface causes the aluminum therest to be dissolved in the electrolyte faster than it can be brought to the surface from the body of the alloy, thus producing a surface impoverishment of the latter, as a result of which the tendency of more electronegative elements to go into solution (as for example iron and silicon) is increased. On the other hand, if an adequate area of contact is maintained between the bath and the anode alloy there is not only less likelihood of such elements going into solution but also greater likelihood of their being reprecipitated by contact with the anode, where the aluminum reprecipitates them and thus prevents them from contaminating the bath. Similarly, the presence of a crust between the bath and the cathode metal diminishes the area of contact between these bodies and thus increases the cathode current density. Unduly high current density here tends to impoverish of aluminum the bath surface in contact with the cathode, with the result that metals other than aluminum (as for example, in the present instance, alkali earth metal and sodium) may be permanently deposited. Under normal conditions, however, such metals when deposited on the cathode are largely re-dissolved at once by secondary reaction with the bath and are replaced by their equivalent of aluminum, except in so far as sodium escapes from the cathode in the form of vapor. The described decrease in the area of conducting contact surface between the bath and the two metallic layers, increases the electrical resistance of the cell; and consequently, since in practice the cells are operated in series on a circuit with substantially constant current, the formation of this shelf crust results in a rise of voltage across the cell terminals and therefore an increase in power consumption in the cell, without increasing the metal output. As previously stated, the formation of the shelf crust is largely due to too high a content of alumina in the bath.

Several methods are available for keeping the alumina content of the bath below the saturation point. For example the top metal (aluminum) can be ladled or tapped off and a portion of the saturated or nearly saturated bath dipped out, liquid or solid alumina-free or deoxidized bath being added to take the place of that which was removed. The resulting mixture will then be well below the saturation point. Or a portion of the top crust can be broken away and removed, whereupon the top crust will reform at the expense of the saturated bath within the cell. New alumina-free or deoxidized bath can be added either in solid or liquid form to take the place of that which

went to form the new top crust. In the first method the saturated bath removed from the cell can be regenerated and prepared for re-entry into the process by crushing it and electrolyzing it in a separate pot for the reduction of the alumina, the de-oxidized bath thus obtained being stored for use when required.

Another method of preventing saturation of the bath with alumina is to de-oxidise the alumina continuously, or from time to time, for example by electrolyzing the bath according to the Hall process of producing aluminum from alumina. This may be accomplished by placing a carbon electrode in contact with the bath and connecting it with the positive terminal of the cell, thus making the carbon electrode an anode. Any current leaving the carbon anode serves to electrolyze alumina in the usual manner, depositing aluminum on the cathode metal, or on the anode metal, or on both, depending upon the voltage used, the oxygen being liberated at the anode and forming  $CO_2$  with a portion of the carbon. The carbon dioxide gas so produced bubbles up through the top metal and may be partially reduced to monoxide but nevertheless serves to carry off some of the oxygen from the bath and therefore to deprive it of alumina, thus decreasing the alumina to a point below saturation. In practice the introduction of a carbon anode into the bath presents some difficulty, for the reason that carbon is lighter than the bath and hence must be forcibly held down in the latter, and for the further reason that any device used for holding the electrode down necessarily passes through the top metal. One way is illustrated in Figs. 1 and 8 of the drawings. In these figures 50 represents a carbon disk into which is threaded a carbon stud 51, into the upper end of which is threaded a water-cooled iron terminal 52. The latter is screwed into the bottom of a pipe 53 which serves to support the terminal and the disk and also to supply the electrolyzing current and the cooling water. At its top the pipe is fitted into the underside of a closed chamber 54 through which a water supply pipe 55 projects down into the pipe and well to the bottom of the latter. Water thus introduced into contact with the iron terminal 52 rises around the pipe 55 and flows out of the chamber 54 by way of pipe 56. The pipe 53 is fastened on a support 57 in such manner as to hold the carbon disk 50 submerged in the bath below the aluminum layer 48. The support 57 is shown as composed of two channel irons arranged back to back. It may be insulated from the frame 38, as indicated at 57<sup>a</sup>. Around the carbon stud 51, water-cooled terminal 52, and the lower end of pipe 53, is an insulating and refractory crust 58 which may consist of a mixture of

bath and corundum previously cast in place. This crust serves to prevent the aluminum top metal from making contact with the carbon disk or with the electrically associated parts, and thereby prevents a short-circuit between the top metal and the de-oxidizing anode. The latter can be supplied with current from an independent source, not shown, or it can be electrically connected with the positive bus 33 in any convenient manner, preferably through a suitable circuit-breaker, not shown, from which current may be carried by means of a cable 59, Fig. 1, connected with the pipe 53. In practical operation it is usually sufficient to de-oxidize the bath intermittently, depending upon the rate (as determined by experience) at which oxygen finds its way into the bath. If the voltage of the de-oxidizing current is sufficiently lower than that of the main current (which is supplied to the carbon bottom of the cell) the former current will flow entirely between the de-oxidizing anode and the cathode aluminum, and the aluminum resulting from de-oxidation of alumina will be deposited mostly if not entirely on the cathode. On the other hand, if the de-oxidizing voltage is higher than the main voltage (between the cell terminals) part, at least, of the de-oxidizing current may flow between the de-oxidizing anode and the metal below the electrolyte, thus depositing some of the aluminum in the latter metal.

Another method of de-oxidizing the electrolyte is to remove the top layer of aluminum and reverse the electrical connections, making the upper electrodes the anode and the layer of metal at the bottom the cathode. Alumina is then reduced as in the Hall process, and when the operation has proceeded as far as desired normal conditions are resumed.

The energy-efficiency in electrolytic processes of refining aluminum is dependent largely upon the perfection of the measures taken for preventing escape of heat. Theoretically almost no energy is required for the refining; but practically, in the absence of some other adequate source of heat, sufficient electrical energy must be expended to maintain the anode, the bath, and the cathode in a fused condition, and consequently the amount of electrical energy which must be supplied is almost exactly the equivalent of the heat permitted to escape. After the heat insulation of the cell has been perfected to the maximum practicable extent, nothing further can be accomplished in limitation of the amount of heat escaping from a heated body of given dimensions, and with the minimum heat-loss the energy input required by the cell will also be a minimum. In the interests of power economy the cell should be operated at the lowest

practicable voltage. Accordingly the electrolyte, which furnishes the major portion of the resistance, should be in as thin a layer as is permissible, and it has been found that 5 a layer from  $2\frac{1}{2}$  to 4 inches thick is in general satisfactory. With a bath or electrolyte of any predetermined workable depth, the current density permissible varies between a lower limit which is sufficient to 10 maintain the anode, the bath and the cathode in a molten state, and an upper limit at which volatilization of the bath is excessive, or at which too large a proportion of anode impurities go into solution. These 15 limits, with the various bath-compositions which have been found practicable, are approximately  $800^{\circ}$  C. and  $1100^{\circ}$  C., respectively, with a preferable working temperature of about  $950^{\circ}$  C. The permissible lower 20 limit of current density also varies inversely with the dimensions of the cell, since the heat loss per unit of volume in a large cell is less than that in a small cell on account of the smaller ratio of heat-dissipating area 25 to the volume.

In a cell having a cross section through the electrolyte of 9.6 square feet it has been found that the preferable current is, in general, 8500 amperes, but that the process is 30 workable with currents between 7500 and 12000 amperes. The preferable current density in a cell having the electrolyte cross-sectional area mentioned is therefore 885 amperes per square foot, with a permissible 35 minimum of about 780 amperes and a permissible maximum of about 1250 amperes, per square foot. With the preferred current density mentioned, the total voltage between 40 the terminals of the cell may be about 6 volts. Larger cells may be operated with lower current densities, and at lower voltages, and by varying the size of the cell, the composition of the bath, the conductivity of 45 the bath, and the effectiveness of the heat insulation, the present electrolytic refining process is workable with current densities between about 500 and about 2500 amperes per square foot of cross section of the bath. In general the lower practical limit of voltage is about 3.5 and the upper limit is of 50 course indefinite.

The current is led from the molten aluminum cathode preferably by means of the electrodes or current-carrying members described in the copending application of Francis C. Frary, Serial No. 672,867 filed November 5, 1923. These are made of graphite, in the form of short, thick rods or cylinders, and may be protected against oxidation in the air by means of a non-oxidizable coating which may consist of molten bath material applied to the rods as a thin layer and allowed to freeze thereon.

Practically any alloy of aluminum which 55 has a density greater than that of the elec-

trolyte and remains sufficiently fluid or mobile throughout the operation, may be refined by our process. Preferably, however, we use an alloy of which the principal components are aluminum and copper.

The layer of aluminum floating on the molten bath or electrolyte should be of sufficient expanse to touch the side lining of the cell around the entire perimeter thereof and should be thick enough to insure firm contact with this lining, in order to prevent or minimize volatilization of the bath, which occurs to a greater or less extent at working temperatures and increases as the temperature rises. On account of the surface tension of molten aluminum the top layer should be of substantial depth, and it is therefore desirable to maintain a thickness of at least two inches at all times.

It is to be understood that the invention is not limited to the details herein specifically illustrated or described but can be carried out in other ways and with other apparatus, without departure from its spirit.

We claim—

1. In the electrolytic refining of aluminum, the steps comprising electrolyzing a molten body of impure metal or alloy containing aluminum, as anode, with a superimposed fused bath containing aluminum fluorid, and removing alumina from the bath as may be necessary to keep the bath unsaturated therewith.

2. In the electrolytic refining of aluminum, the method of maintaining the electrolyte fluid at the operating temperature, which consists in removing oxygen from the electrolyte.

3. In the electrolytic refining of aluminum, the steps comprising electrolyzing with a fused fluorid bath, and treating the bath to maintain the same suitably fluid at the operating temperature.

4. In the electrolytic refining of aluminum, the steps comprising electrolyzing a molten body of impure metal or alloy containing aluminum, as anode, with a superimposed fused bath containing aluminum and sodium fluorids, and removing alumina from the bath as may be necessary to keep the bath unsaturated therewith.

5. In the electrolytic refining of aluminum, the steps comprising electrolyzing with a fused fluorid bath, and treating the bath from time to time to keep it unsaturated with alumina.

6. In the electrolytic refining of aluminum with a fused bath containing aluminum and barium fluorids under conditions causing accumulation of alumina in the bath, the step comprising treating the bath electrolytically from time to time to prevent saturation thereof with alumina.

7. In the electrolytic refining of aluminum with a fused bath containing alumini-

- num and barium fluorids under conditions causing accumulation of alumina in the bath, the step comprising removing alumina from the bath as may be necessary to keep the bath unsaturated therewith.
8. In the electrolytic refining of aluminum with a fused bath containing aluminum and barium fluorids under conditions causing accumulation of alumina in the bath, the steps comprising electrolytically de-oxidizing alumina in the bath and depositing the resulting aluminum on the cathode, to keep the bath unsaturated with alumina.
15. 9. In the electrolytic refining of aluminum with a fused bath containing aluminum, sodium and barium fluorids under conditions causing accumulation of alumina in the bath, the steps comprising electrolytically de-oxidizing alumina in the bath and depositing the resulting aluminum on the cathode, to keep the bath unsaturated with alumina.
25. 10. The method of combined refining and reduction, which consists in electrolytically refining impure metal acting as anode in a fused electrolyte, and reducing material from said electrolyte by current from a carbon electrode immersed in said electrolyte.
30. 11. The method of simultaneous refining and reduction in a single cell, which consists in electrolytically depositing substantially pure metal from a molten anode containing the metal in metallic form, upon a molten cathode in a suitable molten bath, and reducing oxid of said metal from said bath by current from a deoxidizing electrode immersed in said bath, and depositing the metal so produced on said cathode.
40. 12. In electrolytic refining, the steps comprising electrolyzing with an impure metal anode in a bath capable of dissolving oxid of said metal and keeping said bath unsaturated with said oxid by electrolyzing with a carbon anode immersed therein.
45. 13. The method of operating an electrolytic cell which consists in electrolyzing with a soluble electrode and a fused bath to deposit metal from the latter, and also electrolyzing the bath by means of an oxidizable electrode to reduce oxid in said bath.
55. 14. The method of refining aluminum which consists in passing current from a body of molten alloy containing aluminum, as anode, to a molten body of aluminum as cathode, through an intermediate bath of molten electrolyte capable of dissolving alumina whereby aluminum is removed from the anode and deposited on the cathode, and maintaining the fluidity of said bath at working temperature by intermittently removing alumina therefrom.
60. 15. In the electrolytic refining of aluminum, the steps comprising passing current from a body of molten alloy containing aluminum, as anode, to a molten body of aluminum as cathode, through an intermediate bath of molten electrolyte containing aluminum, sodium, and barium fluorids whereby aluminum is removed from the anode metal and deposited on the cathode; and passing from an unfused oxidizable anode through the bath to the molten cathode, to electrolytically deoxidize the alumina in the bath and add the resulting aluminum to the molten cathode.
70. 16. In the electrolytic refining of aluminum, the steps comprising passing current from a body of molten alloy containing aluminum, as anode, to a molten body of aluminum as cathode, through an intermediate molten bath containing aluminum, barium, and sodium fluorids whereby aluminum is removed from the anode metal and deposited on the cathode; and from time to time passing electrolyzing current through the bath to the cathode from a carbon anode in contact with the bath, to deoxidize the alumina in the bath and thereby prevent too great accumulation of alumina therein.
80. 17. In the art of refining by electrolysis, the improvement comprising forming above a molten electrode floated on a molten bath a heat-insulating crust composed at least in part of frozen bath material, and thereafter restricting the thickness of said crust by controlling the composition of said bath.
85. 18. In the art of refining by electrolysis, the improvement comprising electrolyzing a molten bath lying above a molten anode in a cell having heat-insulating side surfaces, and depositing the refined metal on a molten cathode floated on and covering said bath, and establishing above said cathode a heat-insulating crust substantially continuous with said heat-insulating side surfaces whereby volatilization and heat losses are minimized.
90. 19. In the electrolytic refining of aluminum, the steps comprising establishing a lower layer of molten alloy containing aluminum, as anode, an upper layer of molten aluminum as cathode, and an intermediate layer of molten electrolyte containing cryolite and a metal fluorid serving to increase the density of the electrolyte; establishing above the molten aluminum layer a heat-insulating top-crust composed, at least in part, of molten electrolyte coming up from below and freezing above the aluminum; passing current through the three layers mentioned so as to remove aluminum from the lower and add it to the upper layer; and treating the bath to remove alumina, whereby excessive rise of the freezing point of the bath, and consequent excessive thickening of the top-crust, are prevented.
100. 20. In the electrolytic refining of aluminum, the steps comprising establishing a

lower layer of molten alloy containing aluminum, as anode, an upper layer of molten aluminum as cathode, and an intermediate layer of molten electrolyte containing cryolite and a metal fluorid serving to increase the density of the electrolyte; establishing above the molten aluminum layer a heat-insulating top-crust of suitable thickness and composed, at least in part, of molten electrolyte coming up from below and freezing above the aluminum; passing current through the three layers mentioned so as to remove aluminum from the lower and add it to the upper layer; and controlling the composition of the electrolyte to prevent excessive thickening of the top-crust.

21. In the electrolytic refining of aluminum, the steps comprising passing current from a lower layer of molten alloy containing aluminum, as anode, to an upper layer of molten aluminum as cathode, through an intermediate layer of molten electrolyte containing aluminum fluorid; establishing above the molten aluminum layer a heat-insulating top-crust composed, at least in part, of alumina and of molten electrolyte coming up from below and freezing above the aluminum; and controlling the composition of the electrolyte to prevent excessive thickening of the top-crust by progressive freezing of electrolyte thereon.

22. In the electrolytic refining of aluminum, the steps comprising passing current from a lower layer of molten alloy containing aluminum, as anode, to an upper layer of molten aluminum as cathode, through an intermediate layer of molten electrolyte containing aluminum fluorid; establishing above the molten aluminum layer a heat-insulating top-crust composed, at least in part, of molten electrolyte coming up from below and freezing above the aluminum; and controlling the composition of the electrolyte to prevent excessive thickening of the top-crust by progressive freezing of electrolyte thereon.

23. In the electrolytic refining of aluminum, in which molten cathode aluminum, electrolyte, and anode alloy containing aluminum, are arranged in downwardly successive layers, the steps comprising establishing above the top layer a heat-insulating crust of suitable thickness and composed, at least in part, of molten electrolyte coming up from below and freezing above the top layer, and controlling the composition of the electrolyte to prevent excessive thickening of the crust.

24. In the electrolytic refining of aluminum, in which cathode aluminum, electrolyte, and anode alloy, all in the molten state, are arranged in downwardly successive layers, the step comprising establishing above the top layer a heat-insulating crust composed, at least in part, of electrolyte

brought up from below and frozen above the top layer.

25. In the electrolytic refining of aluminum, the steps comprising establishing a molten lower layer of alloy containing aluminum, as anode, an upper cathode layer of molten aluminum, and an intermediate layer of electrolyte containing aluminum, sodium and barium fluorids; establishing above the aluminum layer a heat-insulating top-crust composed, at least in part, of electrolyte coming up from below and freezing above the aluminum; passing current from the anode alloy through the electrolyte to the aluminum cathode; maintaining the electrolyte unsaturated with alumina to prevent excessive thickening of the top-crust; and maintaining the aluminum layer sufficient in expanse to cover the entire layer of electrolyte and thereby diminish volatilization of the latter and escape of sodium vapor to the top-crust.

26. In the electrolytic refining of aluminum, in which cathode aluminum, electrolyte, and anode alloy, all in the molten state, are arranged in downwardly successive layers, the improvement comprising establishing on the aluminum layer a heat-insulating crust of suitable thickness composed, at least in part, of molten electrolyte coming up from below and freezing above the aluminum layer, and maintaining the aluminum layer sufficient in expanse to cover the entire layer of electrolyte and thereby diminish volatilization of the latter.

27. In the electrolytic refining of aluminum, in which cathode aluminum, electrolyte, and anode alloy, all in the molten state, are arranged in downwardly successive layers, the step comprising maintaining the aluminum layer sufficient in expanse to cover the entire layer of electrolyte and thereby diminish volatilization thereof.

28. In the electrolytic refining of aluminum, in which cathode aluminum, electrolyte, and anode alloy, all in the molten state, are arranged in downwardly successive layers in a suitable cell or vessel, the step comprising maintaining the aluminum cathode layer sufficient in depth and expanse to make firm contact with the sides of the cell or vessel and cover the entire layer of electrolyte.

29. In the electrolytic refining of aluminum, in which cathode aluminum, electrolyte, and anode alloy, all in the molten state, are arranged in downwardly successive layers in a suitable cell or vessel, the step comprising maintaining the aluminum cathode layer at least about 2 inches thick and sufficient in expanse to make firm contact with the sides of the cell or vessel and cover the entire layer of electrolyte.

30. In the electrolytic refining of aluminum, in which cathode aluminum, electro-

- lyte, and anode alloy, all in the molten state, are arranged in downwardly successive layers, the step comprising maintaining the aluminum layer sufficient in expanse to cover the entire layer of electrolyte and thereby diminish volatilization thereof, while maintaining around and above the aluminum layer an inclosure composed of frozen electrolyte. 35
- 10 31. In the art of refining by electrolysis, the improvement comprising forming above a molten electrode floated on a molten bath a heat-insulating crust composed at least in part of frozen bath material. 40
- 15 32. In the electrolytic refining of aluminum, the step comprising electrolyzing a fused bath and depositing the separated aluminum on a molten aluminum cathode floating on the electrolyte and completely in- 45
- 20 closed in fused and frozen bath-ingredients. 50
33. In the electrolytic refining of aluminum, the steps comprising electrolyzing a fused bath and depositing the separated aluminum on a molten aluminum cathode 55
- 25 floating on the bath, and maintaining around and above the cathode an inclosure composed of frozen bath-ingredients. 55
34. In the electrolytic refining of aluminum, the steps comprising electrolyzing a 60
- 30 fused bath in contact with molten metallic bodies as anode and cathode; and maintain- 65
- ing adequate area of contact between the fused bath and the molten metallic bodies, and an inclosure composed of frozen bath-ingredients around and above the cathode. 35
35. In the electrolytic refining of aluminum, the steps comprising electrolyzing a fused bath in contact with molten metallic bodies as anode and cathode, and maintaining adequate area of contact between the fused bath and the molten metallic bodies, and above the cathode a heat-insulating crust composed of frozen bath-ingredients. 40
36. In the electrolytic refining of aluminum, the steps comprising electrolyzing a fused bath in contact with a molten aluminum cathode and a molten aluminum-alloy anode, and maintaining adequate area of contact between the fused bath and the anode. 45
37. In the electrolytic refining of aluminum, the steps comprising electrolyzing a fused bath in contact with molten metallic bodies as anode and cathode, and regulating the composition of the bath to prevent formation of crust between the bath and said metallic bodies. 50

In testimony whereof we hereto affix our signatures.

WILLIAM HOOPES.  
FRANCIS C. FRARY.

lyte, and anode alloy, all in the molten state, are arranged in downwardly successive layers, the step comprising maintaining the aluminum layer sufficient in expanse to cover the entire layer of electrolyte and thereby diminish volatilization thereof, while maintaining around and above the aluminum layer an inclosure composed of frozen electrolyte.

10 31. In the art of refining by electrolysis, the improvement comprising forming above a molten electrode floated on a molten bath a heat-insulating crust composed at least in part of frozen bath material.

15 32. In the electrolytic refining of aluminum, the step comprising electrolyzing a fused bath and depositing the separated aluminum on a molten aluminum cathode floating on the electrolyte and completely in-

20 closed in fused and frozen bath-ingredients.

25 33. In the electrolytic refining of aluminum, the steps comprising electrolyzing a fused bath and depositing the separated aluminum on a molten aluminum cathode floating on the bath, and maintaining around and above the cathode an inclosure composed of frozen bath-ingredients.

30 34. In the electrolytic refining of aluminum, the steps comprising electrolyzing a fused bath in contact with molten metallic bodies as anode and cathode; and maintain-

ing adequate area of contact between the fused bath and the molten metallic bodies, and an inclosure composed of frozen bath-ingredients around and above the cathode.

35 35. In the electrolytic refining of aluminum, the steps comprising electrolyzing a fused bath in contact with molten metallic bodies as anode and cathode, and maintaining adequate area of contact between the fused bath and the molten metallic bodies, and above the cathode a heat-insulating crust composed of frozen bath-ingredients.

40 36. In the electrolytic refining of aluminum, the steps comprising electrolyzing a fused bath in contact with a molten aluminum cathode and a molten aluminum-alloy anode, and maintaining adequate area of contact between the fused bath and the anode.

45 37. In the electrolytic refining of aluminum, the steps comprising electrolyzing a fused bath in contact with molten metallic bodies as anode and cathode, and regulating the composition of the bath to prevent formation of crust between the bath and said metallic bodies.

50 In testimony whereof we hereto affix our signatures.

WILLIAM HOOPES.  
FRANCIS C. FRARY.

#### Certificate of Correction.

It is hereby certified that in Letters Patent No. 1,534,319, granted April 21, 1925, upon the application of William Hoopes, of Pittsburgh, and Francis C. Frary, of Oakmont, Pennsylvania, for an improvement in "Refining Aluminum Electrolytically with Fused Electrolytes," an error appears in the printed specification requiring correction as follows: Page 9, line 72, claim 15, after the word "passing" insert the word *current*; and that the said Letters Patent should be read with this correction therein that the same may conform to the record of the case in the Patent Office.

Signed and sealed this 18th day of August, A. D. 1925.

[SEAL]

KARL FENNING,  
Acting Commissioner of Patents.

**Certificate of Correction.**

It is hereby certified that in Letters Patent No. 1,534,319, granted April 21, 1925, upon the application of William Hoopes, of Pittsburgh, and Francis C. Frary, of Oakmont, Pennsylvania, for an improvement in "Refining Aluminum Electrolytically with Fused Electrolytes," an error appears in the printed specification requiring correction as follows: Page 9, line 72, claim 15, after the word "passing" insert the word *current*; and that the said Letters Patent should be read with this correction therein that the same may conform to the record of the case in the Patent Office.

Signed and sealed this 18th day of August, A. D. 1925.

[SEAL.]

**KARL FENNING,**  
*Acting Commissioner of Patents.*